

Sept. 22, 1936.

H. L. BENDER ET AL

2,055,450

WATERPROOF FABRIC AND PRODUCTION THEREOF

Filed Sept. 12, 1931



Fig. 4

Fig. 3

Fig. 2

Inventor

By FRANK L. BENNETT, JR.  
AND HOWARD L. BENDER,  
*Jack Richman* Attorney

## UNITED STATES PATENT OFFICE

2,055,450

WATERPROOF FABRIC AND PRODUCTION  
THEREOF

Howard L. Bender, Bloomfield, and Frank I. Bennett, Jr., Highland Park, N. J., assignors to Johnson & Johnson, New Brunswick, N. J., a corporation of New Jersey

Application September 12, 1931, Serial No. 562,588

5 Claims. (Cl. 91—68)

The invention relates to waterproof fabrics and to the production thereof and more particularly to fabrics whether interstitial or otherwise, such as woven or other textile fabric and fabrics of the nature of paper, which inherently or of themselves are not waterproof and require treatment to make them so; and it provides a waterproof fabric possessed of certain definite, distinctive, and novel characteristics whereby it is susceptible of manifold uses and applications in the industrial arts and sciences.

The waterproof properties of liquid coating compositions such as reaction condensation products having resin characteristics are well known and prior to this invention it has been proposed to make fabrics waterproof by treating them with reactive resinous materials. The liquid coating composition was applied generally by dipping or by spraying and the result was more or less satisfactory where relatively heavy gage or non-uniformity of thickness of the coating was of no moment and where stiffness or tackiness, either manifest or eventual, were not problems.

Attempts to perfect the practice by resort to calendering failed because none of the known materials would lend themselves to known methods of calendering; and so it is that, although the literature fairly abounds with suggestions and examples of resinoid coated cloths or other fabrics, the information has no practical value and the results are abortive in the sense that a careful following out of the specifications and mode of procedure simply results in a stiff composite fabric leaving much to be desired in stability and general appearance.

The nature of the invention resides in the method, and in the product of that method, which in one aspect consists in the selection and treatment of a reactive resin composition to condition it for successful application by calendering or otherwise, and in another aspect consists in the method of calendering, or in short, coordinating the factors of proper coating material and proper application of that material, for the ultimate purpose and result of producing a waterproof fabric, characterized by its marked flexibility, uniformity of gage or thickness, and by its stability and freedom from tackiness over long periods of time regardless of exposure to different temperature conditions.

The invention will be described in connection with the accompanying drawing, forming a part hereof, wherein

Figure 1 is a layout of apparatus suitable for practicing the invention.

Figs. 2 and 3 are plan and sectional views, respectively, of the new fabric; and

Fig. 4 is a sectional view of fabric coated on both sides, either with reactive resin composition, or with one facing of such composition and with the other facing of, for example, the conventional rubber adhesive mass or compound.

10 *The coating material*

In the practice of the invention considerable care and caution should be exercised in preparing the proper coating material and in properly treating the same so that it readily will lend itself to successful application, such as successful calendering, which includes proper filming and freedom from pin holes. The starting material may be such complex compounds formed by reacting fatty oils and fatty acids containing at least one unsaturated bond per molecule with mono phenols, diphenols or polyphenols as phenol, xylenol, resorcinol, etc. in presence of so-called "converting agents" for instance, metallic salts such as iron chloride, acids such as phosphoric acid or sulphuric acid, organic acids such as oxalic acid, natural resins such as rosin and organic liquids as triethyl citrate. These complex compounds act like highly substituted phenolic compounds in that they dissolve in alkaline solutions under proper conditions which vary for each individual compound. However, they all dissolve in saturated sodium hydroxide ethyl alcohol solutions to give sodium salts which can be converted back to the original complex oil-phenol compound by acidification. The complex oil-phenol compounds and fatty acid phenol compounds also are alike in that they all react with aldehydes, such as formaldehyde, benzaldehyde, furfuraldehyde or salicyldehyde or even in such weak aldehydic compounds as some starches and sugars, to form resins. The complex oil-phenol compounds may be mixed with any other phenol and the mixture made into a resinous complex by reacting with aldehydes. These products are soluble in fatty oils so that free fatty oils may be mixed therewith and the mixture made by reaction with aldehydes, or hardening agents, into resinous complexes modified by free oil.

Excellent results have been achieved with a resinous material consisting of 100 parts phenol, 150 parts tung oil, two parts phosphoric acid, which material, in substantially the proportions stated, is refluxed for two hours at about 185 to 55

190° C. more or less. After cooling there is added to it 20 parts, more or less, hexamethylenetetramine, and the mass is then reacted for one hour at 100° C. or to a viscosity of 200 k. v., when a 5 sample is dissolved in an equal weight of toluene. The product when run through a filter press is a soft, sticky, semi-fluid mass having an odor strongly suggestive of ammonia.

10

The reactive product just described, when in the form of a thick viscous varnish will penetrate into fibrous structures and modify their flexibility; on the other hand, when set to a thin jell 15 it no longer penetrates but swells in solvents to give a dry surfaced jelled mass, resembling gelatins in water, which is difficult to knife spread. And, if sufficient solvent combination is used to break the jell structure, the mixture is very dilute 20 and sticky.

The product in this state is unsuitable for calender-coating because, obviously, it is fugitive in the sense that it has a tendency to flow promiscuously due to the presence of solvents and 25 volatiles and the character and extent of its penetration cannot be controlled. However, we have discovered that by a certain and definite treatment we are able to obtain wholly unexpected and remarkable results in phase characteristics and to obtain an end product which can be frictioned to a degree where it can be calender-coated in the form of flexible, thin, coherent sheets or films which are substantially confined to the surface of the fabric. By "substantially 30 confined to the surface" we mean that although the new coating material may and does to a certain extent penetrate into major interstices or voids of the fabric for anchorage purposes it does not penetrate to any substantial extent into 35 minute interfibrous spaces such as between the fibers of the threads or between adjacent fibers at the crossing of the threads of woven fabrics.

According to the conditioning step of our invention, a batch of flexible resinoid material together with from eight to twenty per cent of its 40 weight of filler is worked down, for example, in a suitable mill 5, the rolls of which are heated to about 180° F. The filler may be either of the inert or of the reactive type. Examples of the 45 former are whiting, corn starch, barytes, wood flour, powdered asbestos, and the like inert materials, either alone or in various combinations. Examples of the reactive fillers are zinc oxide, magnesium oxide, lead oxide, aluminum oxide, 50 etc. It is preferred to use the so-called reactive type of filler and, for example, zinc oxide. In fact, we have discovered that the use of a reactive filler has far reaching consequences and makes for a decided advance in the art. The reactive 55 filler eventually combines chemically with either the excess oils in the resin or with the uncombined phenol to form complex organic compounds which might be called phenolates.

It is preferred to use the so-called reactive type 60 of filler and, for example, zinc oxide. The reactive filler eventually combines chemically with either the excess oils in the resin or with the uncombined phenol to form complex organic compounds which might be called phenolates. It 65 has been found that when an ordinary phenol formaldehyde resin is mechanically worked down, as by kneading or milling, with a filler such as zinc oxide, in the presence of heat, until it is more thoroughly combined than it would be in the 70 varnish state, the zinc oxide does not operate to 75

form a harder rubbery mass but is simply dispersed throughout the spongy resinous material the same as any other filler.

The phenol-oil-formaldehyde product should not be allowed to have reached too advanced a state of polymerization before mixing it with the reactive filler because otherwise the oil, phenol and aldehyde may become so combined that no unsaturated bonds remain to hook up with the zinc oxide. 10

The so-called hot mill is operated for about twenty minutes, whereupon the batch is transferred for further and immediate working to the rolls of a so-called cold mill 6, that is to say, a mill operated at about room temperature. The 15 second milling is continued, likewise, for about twenty minutes, or until the material is free from air or gas inclusions and otherwise manifests readiness for calendering.

Hot milling affects both the chemical and 20 physical state of the resinoid in that the resinoid action is slightly advanced on the hot rolls, and the physical condition is such that the resinoid is smooth and has the proper consistency (allowing for the cold rolling) to be calendered onto the 25 cloth. If the resinoid were merely removed from the hot rolls and permitted to stand, the hardening action would possibly proceed to a point where the resinoid would be useless. Therefore, the plastic resinoid mass is removed from the 30 hot rolls and worked on the cold rolls. The cold rolls increase the homogeneity of the resinoid and also stop the chemical hardening action or polymerization of the resinoid so that the mass can be stored until desired for calendering, without 35 chemical hardening.

In using the hot and cold rolls, the mass is merely worked on the hot rolls as above indicated. Then a hot sheet is taken off of the hot rolls and fed by hand or by gravity or other 40 means to the cold rolls where it is further worked and cooled to room temperature. A mass of the unformed amorphous material from the cold rolls is then friction calendered on to a base, such as cloth. 45

#### Calendering

Successful calendering depends largely upon temperature conditions which vary somewhat for each rubbery resinoid so used. Accordingly, for 50 the above example, the top roll of the calender 7 is heated to about 120° F., the bottom roll to about 140° F., the middle roll being maintained at room temperature or from five to ten degrees above it. When the top roll is below 120° F., the material 55 does not sheet well and when it is above that temperature the film presents pin holes, probably due to air or gas inclusions or to a tendency of the material to adhere to the roll. Experiments were tried with the middle roll at less than room temperature and it was found that moisture condensation from the air and from the cloth or other fabric in contact with the hot bottom roll seriously affected the binding of the mass to the 60 cloth. The bottom roll is kept at a higher heat than the middle roll because it was found, that with both at the same temperature, the material had a tendency to transfer to the bottom roll in the space beyond the edges of the cloth. It 65 further developed that moisture in the cloth or other fabric operated detrimentally against uniformity of adhesion of the coating. If only traces of moisture are present, they are removed by the heat of the bottom roll, otherwise 70 75

thorough dryness of the fabric may be insured by resorting to conventional drying facilities.

*Curing*

5 The coated fabric when it leaves the calender is not very tacky and may be rolled upon itself on a regular mill roll. In the above example, in this state, it is not stable for the various commercial purposes for which it is intended. Hence, in 10 order to promote further polymerization, to remove any vestige of tackiness, and to insure a hard enamel surface finish characterized by its uniformity of gage, its smoothness, its resistance to abrasion and its flexibility which for all practical purposes is that of the foundation fabric, the 15 coated material is subjected to heat treatment, as by passing it through a heater 8. It may here be remarked that, for some resinoid mixtures and for certain uses, heating beyond the calender 20 stage is not necessary.

*The product*

It is characteristic of the new product that the cohesion or binding action between the foundation fabric and the coating is of such nature 25 that, as graphically shown in Fig. 3, there is controlled penetration into the interstices or voids of the foundation fabric, generally just sufficient penetration being permitted to hold to the fabric 30 surface and without penetration into the fibers of the fabric itself. We have discovered that penetration between the interlocking fabric fibers results in a sharp drop in flexibility of the fabric itself. This controlled or non-penetration is a 35 valuable attribute and is especially advantageous in cases where it is expedient or desirable to apply a mass or coating to the opposite or rough side of the foundation fabric, for example, a lining for raincoat purposes, or a cement or adhesive such as that employed with surgical tape or 40 plaster, in case the material is to be employed as a tape or plaster or for industrial applications requiring adhesion.

The double coated or double faced fabric is 45 shown in Fig. 4 in which 9 is the waterproof coating and 10 is the other coating whatever it may be. And it may be any suitable coating, without regard to contained solvents, in that it is a further merit of the improved resinoid coating that 50 it is substantially indestructible when wetted with or otherwise exposed to chemicals such as encountered daily in the arts, trades and professions; and equally important it is compatible with the conventional rubber adhesive mass such as employed in the manufacture of surgical tapes. 55 in this connection it here may be remarked that the impregnated tape of our invention is distinguished from known products in this, that the

adhesive will adhere in one condition and will not adhere in another condition, that is to say, the adhesive will adhere to the phenolic resinoid before either the one or the other is cured but will not adhere after curing and so the finished 5 tape can be rolled upon itself or stacked.

Having described the invention, what is claimed is:—

1. The new fabric embodying porous foundation material and a flexible calendered coat comprising the reaction product of an oil soluble phenol-oil-aldehyde resinous complex and a substance adapted to render it into a plastic rubber-like mass whereby the coat is manifested as a thin coherent film substantially confined to the 15 surface to which it is applied.

2. The new fabric embodying sheeted porous foundation material and a flexible heat cured calendered coat covering an area thereof and comprising the reaction product of an oil soluble 20 phenol-oil-aldehyde resinous complex and a substance adapted to render it into a plastic rubber-like mass whereby the coat is manifested as a thin coherent film substantially confined to the 25 surface of the area to which it is applied.

3. The new fabric embodying flexible sheeted porous foundation material and a flexible heat cured calendered coat covering an area of one side thereof and comprising the reaction product of an oil soluble phenol-oil-aldehyde resinous complex and a substance adapted to render it into a plastic rubber-like mass whereby the coat is manifested as a thin coherent film substantially confined to the 30 surface to which it is applied, and another coat of material compatible with the 35 calendered coat and covering an area of the opposite side of the fabric.

4. Woven fabric having as an integral part thereof a water, heat and chemical resisting calendered coat which does not appreciably impair the inherent flexibility of the fabric, said coat comprising the reaction product of an oil soluble phenol-oil-aldehyde resinous complex and a substance adapted to render it into a plastic rubber-like mass whereby the coat is manifested as a thin coherent film substantially confined to the 40 surface of the fabric.

5. The new fabric embodying porous foundation material and a flexible calendered coat comprising the heat hardened reaction product of an 50 oil soluble phenol-oil-aldehyde resinous complex and a substance adapted to render it into a plastic rubber-like mass whereby the coat is manifested as a thin coherent film substantially confined to the 55 surface of the fabric, and normally tacky adhesive material on the other side of the fabric.

HOWARD L. BENDER.  
FRANK I. BENNETT, JR.